

## UNITED STATES PATENT OFFICE

2,387,170

## LOW TEMPERATURE LUBRICANTS

John D. Morgan, South Orange, N. J., assignor to  
 Cities Service Oil Company, New York, N. Y.,  
 a corporation of Pennsylvania

No Drawing. Application August 27, 1942,  
 Serial No. 456,366

11 Claims. (Cl. 252—36)

This invention relates to low temperature lubricants. More particularly the invention relates to lubricants made from synthetic compounds which have proper physical properties for low temperature lubrication.

I have discovered that Decalin ( $C_{10}H_{18}$ ), decahydronaphthalene, and Tetralin, tetrahydronaphthalene ( $C_{10}H_{12}$ ), have good lubricating characteristics. Decalin has a boiling point of 379° F. and a freezing point below —55° F. Tetralin has a boiling point of 404° F. and a freezing point below —40° F. Both of these are colorless liquids and have better lubricating characteristics than a neutral mineral oil lubricant, that is a neutral oil having a viscosity of 100 at 100° F. However, if 1% of one of the well known extreme pressure additives is added to Tetralin and Decalin, lubricants of high load-carrying characteristics will be formed.

Decalin has the following viscosities:

| Temperature, ° F. | Viscosity, centistokes |
|-------------------|------------------------|
| —40               | 19.8                   |
| 0                 | 9.5                    |
| 100               | 2.28                   |
| 200               | 1.11                   |

Tetralin has the following viscosities:

| Temperature, ° F. | Viscosity, centistokes |
|-------------------|------------------------|
| —40               | Viscous                |
| 0                 | 6.98                   |
| 100               | 1.68                   |
| 200               | .88                    |

With these viscosity values it is apparent that the viscosity temperature curves are practically flat and therefore there is little change in the temperature range in which a lubricant ordinarily is operative. Due to the fact that the viscosities are so low at the low temperatures, Tetralin and Decalin are well adapted for low temperature lubrication.

Decalin and Tetralin are compatible with the alkali and alkaline earth metal soaps for the production of greases which stay in stable emulsion. The lithium, calcium and aluminum soaps are mutually soluble in Tetralin and Decalin. Preferably the metal soaps are stearates but the oleates and palmitates will blend with Decalin to form good greases. It has been found that from 4 to 20% of these metal soaps may be blended

with Tetralin or Decalin to produce satisfactory greases. It is preferred furthermore to add an extreme pressure additive to the Tetralin or Decalin before they are blended with the soap in making the greases; for example, from 0.1% to 1% of the additive, thereby producing greases having extreme pressure load-carrying characteristics.

Tetralin and Decalin have a tendency to oxidize but it has been found that if a small proportion of from .01% to 0.1% of one of the well known antioxidants is dissolved in the Tetralin or Decalin they become very stable. For example from .01 to .1% of hydroquinone, pyrogallol, or  $\alpha$ -naphthol are very effective antioxidants for stabilizing Decalin and Tetralin.

The extreme pressure additives which may be used with Tetralin and Decalin may be any of the well known additives that are commonly used for treatment of mineral oil lubricants. A small proportion of the extreme pressure additive or agent, for example, from 0.1% to 1%, is effective to impart extreme pressure properties to the lubricant. "Polane," a commercial extreme pressure agent which is known as chloromethyl stearate may be used. Tricresyl phosphite or a mixture of tricresyl phosphite and tricresyl phosphate are effective additives. The sulfurized tricresyl phosphine extreme pressure agents described in Engel Patent No. 2,260,303, granted October 28, 1941, may be used, as also the sulfurized tin salts of alkyl phenol carboxylic acids as described in Patents Nos. 2,197,834-5; 2,256,441; and 2,257,751.

When making the greases the extreme pressure additive and the antioxidant are dissolved in Decalin or Tetralin, and then the treated hydro-naphthalenes are blended with the soaps of lithium, calcium, or aluminum. Preferably the aluminum soap is used in conjunction with the calcium or lithium soaps. A preferred product comprises from 4% to 15% of lithium stearate, from 1% to 3% of aluminum stearate, from 0.1% to 1% of "Polane," from 0.01% to 0.1% of pyrogallol, the remainder of the product consisting essentially of Decalin or Tetralin. Other greases may be made containing from 4% to 20% of a metal soap of a fatty acid such as lithium stearate or one of the other soaps mentioned above, the remainder of such greases consisting essentially of Decalin or Tetralin. These greases may contain a small proportion of an antioxidant or a small proportion of an extreme pressure agent, or both.

Decalin and Tetralin may be mixed together in

most any desired proportion for use as a lubricant, or for use in making a grease which may contain from 4% to 20% of a soap such as lithium stearate.

Decalin and Tetralin are formed by the hydrogenation of naphthalene. The hydrogenation of naphthalene to form Decalin can be carried out to form isomeric compounds, the cis- and trans-Decalins. Each of these isomers may be used as a lubricant. All of the polyhydronaphthalenes tested have been found to have lubricating properties, and the extreme pressure additives are soluble in all of the polyhydronaphthalenes to provide extreme pressure lubricants. The polyhydronaphthalene lubricants may contain from 0.1% to 1% of an extreme pressure agent, or from 0.01% to 0.1% of an antioxidant, or both an extreme pressure agent and an antioxidant in about these proportions.

The preferred form of the invention having been thus described, what is claimed as new is:

1. A low temperature lubricant consisting essentially of a polyhydronaphthalene having dissolved therein a small proportion of an extreme pressure agent sufficient to impart extreme pressure properties to the lubricant.

2. A low temperature lubricant consisting essentially of a polyhydronaphthalene having dissolved therein a small proportion of an extreme pressure agent and a small proportion of an antioxidant, said agent and antioxidant being present in sufficient proportion to respectively impart extreme pressure properties to the lubricant and to protect the lubricant against oxidation.

3. A low temperature lubricant consisting essentially of Decalin having dissolved therein a small proportion of an extreme pressure agent sufficient to impart extreme pressure properties to the lubricant.

4. A low temperature lubricant consisting essentially of Tetralin having dissolved therein a small proportion of an extreme pressure agent sufficient to impart extreme pressure properties to the lubricant.

5. A low temperature lubricant consisting essentially of a mixture of Decalin and Tetralin having dissolved therein a small proportion of an extreme pressure agent sufficient to impart extreme pressure properties to the lubricant.

6. A low temperature lubricant comprising from about 4% to 20% of a metal soap of a fatty acid, the remainder of the lubricant consisting essentially of Decalin.

7. A low temperature lubricant comprising from about 4% to 20% of a metal soap of a fatty acid, the remainder of the lubricant consisting essentially of Tetralin.

8. A low temperature lubricant comprising from about 4% to 20% of lithium stearate, the remainder of the lubricant consisting essentially of Decalin.

9. A low temperature lubricant comprising from about 4% to 20% of lithium stearate, the remainder of the lubricant consisting essentially of Tetralin.

10. A low temperature lubricant comprising from about 4% to 20% of lithium stearate, the remainder of the lubricant consisting essentially of a mixture of Decalin and Tetralin.

11. A low temperature lubricant comprising from about 4% to 15% of lithium stearate, from about 1% to 3% of aluminum stearate, the remainder of the lubricant consisting essentially of Decalin.

JOHN D. MORGAN.